

## UNITED STATES PATENT OFFICE

ELTON R. DARLING, OF DECATUR, ILLINOIS, ASSIGNEE, BY MESNE ASSIGNMENTS, TO  
CORNSTALK PRODUCTS COMPANY, INC., OF NEW YORK, N. Y., A CORPORATION OF  
DELAWARE

PROCESS FOR THE PREPARATION OF PARCHMENT-PAPER STOCK FROM CORNSTALK  
PITH

No Drawing. Application filed October 19, 1928. Serial No. 313,632.

This invention relates to a process for the manufacture of parchment paper stock from cornstalk pith. While this process could be used to advantage on piths from vegetable growths other than cornstalks, for economic as well as physical reasons it has been demonstrated that cornstalk pith has many points of superiority which make it desirable to use same.

10 The step of recovering the pith from the cornstalks is well known and does not constitute in itself a part of this invention. Cornstalk pith is washed from the plant with fibrovascular fibers which closely adhere to 15 the pith and are consequently found meshed therewith as it is commercially produced.

The pith is first subjected to a washing operation by which all dirt and foreign matter is removed. The washed and cleansed pith 20 is then subjected to a digestion operation in water and under heat and pressure such as is set forth in my previous patent application Serial No. 287,651, filed June 22, 1928.

In the course of this digestion operation 25 the pithy mass separates from the fibrovascular fibres, and in the pulpy mass remaining when the digestion is completed the said fibre will be disengaged from but mixed with the pith.

30 This pulpy mass is then washed and conveyed onto flat agitated screens of a mesh that will permit the pulpy pith mass to pass through, the stringy fibrovascular fibres being retained and separated from the pith.

35 The pith then may be bleached by any of the known methods. I have described that the aforesaid pith, either before or after bleaching, is capable of mechanical hydration forming a somewhat gelatinized material which lends itself to the manufacture of 40 parchment paper.

To accomplish this hydration following the bleaching step the material is placed in a beater where it is mixed with water heated to 45 about one hundred and thirty-five degrees

Fahrenheit until hydration is complete when it may be made by any of the known methods into paper of a superior parchment type. The completion of the hydration is most readily detected by one who has become familiar 50 with the operation, and is versed in the art. As for example, by taking samples periodically during the operation and forming therefrom small test sheets until the pulp yields to the desired results. The hydrated pith is 55

now in condition to be converted into paper by being run through a conventional paper machine forming what is known as vegetable parchment. This is to be distinguished from the type of vegetable parchment where cellulose is chemically hydrated by means of sulphuric acid and subsequent washing. What I am producing is what is sometimes known as genuine vegetable parchment.

It is obvious that the temperature of one 65 hundred and thirty-five degrees Fahrenheit given above for the water used in the heating operation may be varied to meet the immediate conditions of the operation.

I claim:—

1. The process for the preparation of parchment paper stock from cornstalk pith which comprises cleansing said pith of foreign matter contained therein, subjecting the cleansed pith to a digesting operation in 75 water under heat and pressure to separate the pith into fibrous and non-fibrous constituents, filtering off the fibrous constituents, bleaching the pithy constituents, and thereupon hydrating the pith by agitating the 80 same with water at 135° F.

2. The process of preparing parchment paper stock from cornstalk pith which comprises cleansing said pith of foreign matter retained therein, softening said cleansed pith by digesting the same in water and causing it to separate into free pith and into fibrous material, separating said fibrous material from said pith, while discarding said fibrous material and retaining said pith, bleaching the 85 90

pith and thereupon hydrating the same by violent agitation at 135° F.

3. The process of treating cornstalk pith which comprises digesting the same to cause separation thereof into free pith and fibro-vascular material and thereafter separating said fibrovascular fibers from the pith and subsequently hydrating the latter in water at 135° F.

10 In testimony whereof I have hereunto affixed my signature.

**ELTON R. DARLING.**